

## UNITED STATES PATENT OFFICE

2,206,616

OSMIUM COMPOSITION AND METHOD OF  
MAKING SAMEAndrew R. Devereux, Chicago, and Carl  
Pfanstiehl, Highland Park, Ill.No Drawing. Application September 17, 1938,  
Serial No. 230,506

14 Claims. (Cl. 75—22)

This invention relates to a method of preparing a new osmium composition.

Osmium is a very difficult metal with which to work. It has tremendous ability to resist wear but on the other hand is extremely brittle and friable and when alloyed in considerable proportions with other metals tends to make them likewise brittle and hard. Various methods have heretofore been suggested for forming alloys of osmium into useful forms and particularly for reducing the brittleness thereof. In all of these cases, however, the osmium has been melted with the alloying metal or metals with the result that the body of the alloy is an osmium alloy of relatively low wear resistance and generally of considerable hardness and brittleness.

In accordance with the present invention the osmium is maintained substantially in its original unmelted or pure form and is bonded together by relatively low melting point metal which is fluxed at a high temperature, but substantially below the melting point of osmium.

The bonding metals employed for pen point use are preferably chosen from the platinum group, platinum being particularly preferred. These metals wet the osmium most readily and at the same time have high corrosion-resistance, high melting point and also are relatively wear-resistant compared with many other metals.

Base metals may be added to the platinum group metal or for some purposes may be employed by themselves. In those instances where high corrosion-resistance is essential, as in connection with pen points, the base metal should be employed in such proportions that the precious metal such as platinum or ruthenium will completely cloak the ordinary lack of corrosion-resistance of the base metal.

In preparing the composition, finely divided, essentially pure osmium metal and finely divided base metal or alloys thereof are mixed. For example, 85 parts of metallic osmium are finely ground in a ball mill to a particle size of 40 microns or less. The grinding is preferably carried on in the presence of a wetting agent and after this has been evaporated the ground powder was mixed with platinum or a platinum yielding compound such as an alcoholic solution of platinum chloride. The alcohol is evaporated leaving a coating of platinum chloride upon the osmium particles.

This mixture is reduced at 1800 to 1900° F. in an atmosphere of hydrogen, leaving a coating of platinum upon the osmium and reducing any osmium oxide present. Ordinarily the reducing

operation is carried on from one to one and one-half hours.

After the reduction is complete the powders are cooled say to 800° F. in an atmosphere of hydrogen and then cooled in an inert gas such as carbon dioxide in order to prevent absorption of hydrogen by the platinum.

The resulting material is then lightly ground in a mortar or ball mill in order to break up any clusters which may have formed and is then formed into particles of predetermined size and shape by pressing in a die.

It is important that the particles be pressed as nearly as possible into the form which they are ultimately to have. For instance, a phonograph needle point may be shaped at this stage as near to the form of the tip of the needle as possible. Preferably, a sharp cone is produced. Similarly, with a pen point the material may be pressed into a sphere or a rectangular block, preferably the latter.

This forms coherent granules which are then given a preliminary heat treatment at say 2600° F. in an inert gas in order to make them somewhat more tough and less likely to break upon handling.

The granules are then heated to about 2000° F. in a vacuum for 15 minutes in order to remove the hydrogen and they are then heated at a temperature above 2600° F., preferably 2700 to 2800° F., for 2 to 4 hours in an inert atmosphere.

They are then cooled from 1400 to 1500° F., the inert atmosphere replaced by hydrogen, and the temperature raised to approximately 2600° F. The granules are maintained for a prolonged period at this temperature in an atmosphere of flowing hydrogen. The time is preferably at least 6 hours and normally from 12 to 18 hours. The flowing hydrogen acts as a gaseous flux and the treatment greatly improves the wear resistance of the granules with respect to relatively soft abrasives.

Prior to the final heat treatment the granules are very wear resistant with respect to hard abrasives, such as emery, and are relatively less resistant to such abrasives as sandpaper or ordinary writing paper. The final heat treatment does not affect the wear resistance with respect to emery but markedly increases it with respect to sandpaper and ordinary writing paper.

The final heat treatment has the peculiar effect of making the material markedly magnetic, even though the presence of ordinarily magnetic metals be avoided so far as practicable. Gran-

ules of 85% osmium, 15% platinum, containing only such iron or nickel impurities, if any, as are normally present in commercially pure osmium, which has been ball milled as here described, 5 were very highly magnetic following the heat treatment.

Boiling the osmium in hydrochloric acid to free it from iron before the mixing or heat treatment did not alter its magnetic properties. Before the boiling it contained approximately .75% of iron.

The magnetic properties are of considerable value, particularly in certain operations such as welding, where the magnetic character of the 15 metal is of great assistance in manipulation.

The platinum may be replaced in part by iron group metals such as nickel, iron or cobalt. For example, a granule containing 85% osmium, 10% platinum, and 5% nickel may be produced by 20 this process.

The platinum may also be replaced in whole or in part by other platinum group metals. For example, a very satisfactory alloy was made which included 25 85% osmium, 10% platinum and 5% rhodium. In this case the preheating with hydrogen was carried on at 2600° F., the treatment in an inert atmosphere from 3000 to 3100° F., and the final treatment in flowing hydrogen at about 2600° F.

30 An alloy of 85% osmium, 10% ruthenium and 5% platinum was preheated at 2600° F., then heated in an inert atmosphere at 2800 to 3000° F. and then in flowing hydrogen at about 2600° F.

In all cases the amount of osmium should 35 predominate. If the amount of other metal is below 10% there is a tendency for the resulting granule to become brittle, whereas above 20% there is a tendency for porosity to develop which becomes undesirable for some purposes when the amount 40 of osmium is below 70%.

For many purposes the final wear resistance improving step may be dispensed with. For example, with phonograph needles the character 45 of wear resistance encountered is specific and it is frequently not necessary to employ the final heating operation.

For example, a granule containing 85 parts 50 osmium, 12½ parts of ruthenium and 2½ parts of nickel may be prepared by heating the pressed powders at approximately 3100° F. for 1 hour. At temperatures of 3200° F. and above the osmium composition becomes hard and brittle. At temperatures of 2700° F. and upwards heating for 3 hours produces fair results. Even at 2600° F. 55 some binding can be secured but the wear is relatively poor. With this mixture very good results were obtained by heating at 2900° F. for 2½ to 3½ hours.

All temperatures are approximate because of 60 the extreme difficulty of accurate measurement at these ranges.

In a similar composition in which the nickel is replaced by more ruthenium so that the resultant composition contains 85 parts of osmium and 15 parts of ruthenium, the temperature range 65 is slightly different. For this mixture the preferred range is 2800° F. to 3200° F., with best results being procured at 3200° F. or slightly below. At 2700° F. and below the metal does not 70 consolidate well.

With higher proportions of nickel as, for example, 85 parts of osmium, 10 parts of ruthenium and 5 parts of nickel, lower temperatures than with the first example are preferred. However, 75 with proportions of nickel in this range the nickel

does not apparently completely dissolve in the ruthenium with the result that the resultant composition is not so corrosion-resistant. It is, however, extremely wear-resistant and is of great value for uses where corrosion is not important, such as phonograph needles. 5

The substitution of platinum for ruthenium raised the temperature range somewhat.

With a 1 to 2 hour heat treatment, 3400° F. is too high for satisfactory results and 3300° F. is 10 somewhat dangerous. Temperatures below 2800° F. are not particularly good.

Strangely enough, with all of these compositions the Brinell or Rockwell hardness of the composition goes down as the heat treatment increases, but the wear resistance of the metal greatly increases. The resulting composition is therefore relatively soft compared to fused osmium alloys of the same composition, but has extraordinarily great wear-resistance. 15 20

The resulting material consists of discrete unmelted small particles bonded together by a flux of lower melting point metal. The osmium particles are apparently in substantially pure form and apparently little of the osmium is dissolved 25 in the flux in substantial amounts.

Preferably the bonding agent predominantly comprises one or more metals of the platinum group other than osmium. This may be platinum, ruthenium, rhodium, palladium, or iridium, 30 although the former two are preferred for most purposes. Other metals such as molybdenum, tungsten, nickel, cobalt, iron, or the like, may be incorporated. For pen point purposes the amounts of these base metals should be low 35 enough, as heretofore explained, that they will completely be cloaked by the platinum group metal. For purposes not requiring such high corrosion-resistance this necessity does not exist and the bonding agent may be made of base metals 40 to a much higher degree or may consist entirely of base metals.

While the bonding material is referred to as relatively low melting point, it is preferable that it have a melting point not too far below that of 45 osmium inasmuch as it is desirable to heat the flux to a point where it will readily wet the osmium and it is not desirable that it be too thin or have a substantial vapor pressure when it reaches such temperatures. 50

There is no objection to minor amounts of 55 modifying agents in the fluxing material. Even for pen point uses, minor amounts of such metals as beryllium, zirconium, tantalum, or columbium may be added if desired. The amount of osmium may be varied over a considerable range, but maximum wear-resistance tends to develop as the proportion of osmium is increased and the proportion of binder is correspondingly reduced to the minimum necessary for binding purposes 60

For all high wear-resistance work, it is preferred that the amount of osmium exceed 50%, and preferably 70%.

The osmium metal employed is preferably pure, but it may have minor amounts of other metals 65 or impurities. The osmium may have been melted prior to incorporation in the present composition.

The foregoing detailed description has been given for clearness of understanding only, and no unnecessary limitations should be understood 70 therefrom, but the appended claims should be construed as broadly as permissible in view of the prior art.

We claim:

1. The method of preparing a relatively soft, 75

- tough high wear resistant osmium composition which comprises mixing osmium in substantially pure finely divided form with a minor proportion of finely divided lower melting point metal, pressing the finely divided material together to form a mass at least loosely coherent, and heating the mass first to produce a hard material of low wear resistance and then continuing the treatment to lower the hardness and increase the wear resistance by fluxing lower melting point metal without fluxing or dissolving any substantial proportion of the osmium. 5
2. The method as set forth in claim 1, in which the flux consists predominantly of platinum group metal of lower melting point than osmium and the heat treating temperature is above approximately 2600° F. and below 3400° F. 10
3. The method which comprises mixing osmium in substantially pure finely divided form with a minor proportion of finely divided metal of lower melting point than osmium, pressing the finely divided material to form a mass at least loosely coherent, and heating the mass for a prolonged period at a temperature in the range of 2600° F. 15 to 3400° F. to produce a tough, highly wear resistant osmium compound in which the osmium is in the form of substantially pure, discrete, minute particles bonded together by a binder of the other metal. 20
4. The method which comprises mixing a major proportion of finely divided osmium and a minor proportion of finely divided lower melting point metal, including platinum group metal other than osmium, consolidating the mixed powders without melting the consolidated material, heat-treating the consolidated material without melting to produce a tough, wear resistant composition, and then further heat treating the material in the presence of gaseous hydrogen at a temperature of the order of about 2600° F. for a prolonged period whereby the wear resistance of the composition to relatively soft abrasives is increased. 25
5. The method as set forth in claim 4, in which the composition of the material includes 70 to 90% osmium and at least 10% of other platinum group metal. 30
6. A tough, wear resistant, osmium composition, comprising approximately 85% osmium in the form of substantially pure, discrete, minute particles bonded together by 15% of a flux predominantly composed of platinum group metal other than osmium and produced by the process of claim 1. 35
7. A tough, wear-resistant, osmium composition, comprising from 70% to 90% of osmium and at least 10% of other platinum group metal prepared by the process of claim 1. 40
8. A sintered, unmelted, composition consisting essentially of 85 parts of osmium, 12½ parts of ruthenium and 2½ parts of nickel prepared by the process of claim 1. 5
9. A tough, wear resistant, osmium composition comprising a predominant proportion of osmium in discrete, minute particles bonded together by a flux having a melting point lower than but approaching the melting point of osmium, the composition having been prepared by the process of claim 1. 10
10. A tough, wear resistant, osmium composition comprising a predominant proportion of osmium in discrete, minute particles bonded together by a flux predominantly composed of platinum group metal other than osmium, and produced by the process of claim 1. 15
11. A tough, wear resistant, osmium composition comprising a predominant proportion of osmium in discrete, minute particles bonded together by a flux predominantly composed of platinum, and produced by the process of claim 1. 20
12. A tough, wear resistant, osmium composition comprising a predominant proportion of osmium in discrete, minute particles bonded together by a flux predominantly composed of ruthenium, and produced by the process of claim 1. 25
13. A tough, wear resistant, osmium composition comprising a predominant proportion of osmium in discrete, minute particles bonded together by a flux comprising 10 to 12½ parts of metal of the class consisting of platinum and ruthenium together with approximately 2½ to 5 parts of a base metal, the composition having been produced by the process of claim 1. 30
14. A tough, wear resistant, osmium composition comprising a predominant proportion of osmium in discrete, minute particles bonded together by a flux comprising 10 to 12½ parts of metal of the class consisting of platinum and ruthenium together with approximately 2½ to 5 parts of metal of the class consisting of nickel, cobalt and iron, the composition having been produced by the process of claim 1. 35

50  
ANDREW R. DEVEREUX.  
CARL PFANSTIEHL.